

# UNITED STATES PATENT OFFICE.

RUFUS N. MOORE, OF THORP SPRING, TEXAS.

## PROCESS FOR TANNING HIDES.

1,256,718.

Specification of Letters Patent. Patented Feb. 19, 1918.

No Drawing.

Application filed December 1, 1916. Serial No. 134,358.

To all whom it may concern:

Be it known that I, RUFUS N. MOORE, a citizen of the United States of America, residing at Thorp Spring, in the county of 5 Hood and State of Texas, have invented a certain new and useful Process for Tanning Hides, of which the following is a specification.

This invention relates to a new and useful 10 form of process and method for preserving, tanning and curing animal hides, such as the tanning of cow, horse and other animal hides preparing them ready for the market and rendering them of commercial value.

15 A purpose of this invention and discovery is to provide such a simplified process and effective method for the purposes described that the stock raisers, farmers and others who may have hides for commercial 20 purposes may quickly and cheaply tan their own hides and obtain a superior grade of leather obviating the necessity of sending their products to tanneries and experiencing that necessary delay and expense which thus 25 attends the preserving of the hide.

In my process I first remove all fatty matter and flesh strips which may have remained on the hide or pelt when same was skinned or removed from the animal. If 30 the hide is green or fresh, and flexible and pliable this removal of the fatty matter is an easy step, but if the hide is dry and has not been recently removed from the animal it should be soaked in water until it is soft 35 and pliable.

Next the pelt or hide is immersed and soaked in a solution of lime water, which step in the process is taken to kill the hair follicle which allows the hair to be easily 40 removed from the hide. After the hair covering, fleshy matter and other foreign substances are entirely removed therefrom it is thoroughly soaked and washed in clear water of several changes till all the lime is thoroughly expunged from the cells of the hide, at which time it is ready to be passed 45 through the primary step of tanning and curing.

This invention proper includes a certain 50 combination and proportion of chemical ingredients composing the tanning solution or ooze. The tanning solution consists of two pounds of gum gambier, one pound of Epsom salts, one pound pulverized alum, 55 and one pound nitrate of sodium all thoroughly dissolved in water raised to an ab-

normal temperature or to a temperature not too hot to be worked with the hands of the tanner. The above described chemical ingredients in the proportions recited are precipitated in water of sufficient quantity to cover a hide of ordinary size. For larger 60 hides the solution or tanning ooze as described will be proportionately increased both in chemical ingredients and warm 65 water.

The hide is now dipped in the tanning ooze and thoroughly saturated and removed, and aired for five minutes after which it is returned to the vessel containing the solution. The hide is next removed and aired 70 two or three times during the first two or three hours of its immersion in the tanning ooze, after which it will be aired one time 75 each succeeding day for two days, thereafter being allowed to remain in said tanning ooze or solution until the hide is thoroughly tanned which requires several days.

The removal and airing process herein described as performed several times during 80 the early stages of the immersion of the hide, or the pelt in the tanning ooze is for the purpose of allowing the tanning solution to be drained and dripped from the hide which will allow the air to penetrate the 85 fiber and formation of the pelt, which action of the air upon the pelt properly expands the inter-fibrillar spaces to a substantially normal size allowing an equal and even distribution and absorption of the solution into 90 the pelt, all of which makes for the better and more even curing process both in coloring and in the tanning thereof.

After the hide remains in the tanning solution for several days and is thoroughly 95 cured and tanned it is removed therefrom and put through another thorough washing in clear water. Another solution is now prepared consisting of one-half ounce of oil of cedar wood, thoroughly mixed in a quantity 100 of water sufficient to cover the hide. The hide is placed in this oil solution and allowed to remain for about twelve hours, after which it is removed and spread out 105 upon a smooth surface in the shade where the superfluous quantity of water contained in the hide is wiped or brushed therefrom. After the hide is partially dried in the shade it is thoroughly oiled with fish oil or other good leather oil, the oil being thoroughly 110 rubbed and absorbed by said hide. After the pelt is thoroughly oiled and further dried

it is given the breaking process which consists of putting the pelt through a rolling and kneading exercise which renders it thoroughly pliable and workable and perfects the tanning and curing process and renders the hide of a commercial value ready for such purposes.

The thorough tanning and curing of a hide as herein described and by the present invention in its described process requires 10 three to twelve days, the time varying according to the size, weight and thickness of the hide.

In the present invention and process of 15 tanning the gum gambier acts as a coloring and preserving agent while the nitrate of sodium permeates the cellular formation of the hide opening the pores and raising the leather till it is slightly thicker and tougher 20 than in its original condition. The alum included in the tanning formula serves to remove the glue or fatty portions of flesh which might have adhered to the pelt after the flesh removing process. The Epsom 25 salts operates on the formation and fiber of the leather to fasten between the fiber of the leather and prevent it from becoming hard

and brittle, which hardness and brittleness might otherwise be caused by the alum; the salts in fact serving to counteract the hardening tendency of the alum.

This process of hide and pelt tanning is simplified in its various steps and will produce a superior form of leather, anyone being able to carry out to a successful termination the tanning of the pelt or hide by the use of the said process.

Having thoroughly described my discovery and invention which resides in the steps and methods taken in curing as heretofore 40 described and as included in the certain combination of chemical ingredients as set up in this instrument of Letters Patent, I now make the following claim therefor:

A tanning solution composed of two 45 pounds of gum gambier, one pound of Epsom salts, one pound of pulverized alum, one pound of nitrate of sodium, and water.

In testimony whereof I affix my signature in the presence of two witnesses.

RUFUS N. MOORE.

Witnesses:

J. M. KENNER,  
W. H. HOLDEN.

Copies of this patent may be obtained for five cents each, by addressing the "Commissioner of Patents, Washington, D. C."